

## UNITED STATES PATENT OFFICE

2,181,143

## MOTOR FUEL

Ernest M. Marks, Lansdowne, Pa., assignor to  
 The Atlantic Refining Company, Philadelphia,  
 Pa., a corporation of Pennsylvania

No Drawing. Application November 12, 1936,  
 Serial No. 110,474

4 Claims. (Cl. 44—9)

The present invention relates to motor fuels, and relates more particularly to motor fuels comprising the oxidation products of iso-olefine polymers such as tri-isobutylene and/or hydrocarbon mixtures containing oxidation products of tri-isobutylene.

A principal object of this invention is the improvement of the anti-detonation characteristics of hydrocarbon motor fuels by the addition thereto of oxidation products of tri-isobutylene.

A further object of this invention is the improvement of the anti-detonation value of motor gasoline by the addition thereto of oxidation products of tri-isobutylene of such boiling range or volatility as not to alter the boiling range of the gasoline to an undesirable extent.

It has been found that tri-isobutylene, per se, is capable of improving the anti-detonation value of motor fuels when added thereto in appreciable quantities, for example, of the order of 10% to 50% by volume. However, since tri-isobutylene is relatively high boiling (355° F.), the addition of substantial quantities thereof to motor fuels within the gasoline boiling range (90° F. to 390° F.) alters the boiling range or volatility of the fuel to an undesirable extent. In other words, the addition of tri-isobutylene to a marketable gasoline having a specified boiling range increases the percentage of the higher boiling components in such fuel to such an extent that the volatility thereof is markedly impaired.

I have discovered that tri-isobutylene may be converted into products more suitable as motor fuel or as addition agents to improve the anti-detonation qualities of motor fuels such as gasoline, by a relatively inexpensive and readily operable process involving oxidation. The products formed by the oxidation of tri-isobutylene not only possess good anti-detonation values but are of such boiling range or volatility as to be compatible with gasolines having definite specifications with respect thereto.

In accordance with my invention, tri-isobutylene is subjected to the action of an oxidizing medium such as air, oxygen or gaseous mixtures containing oxygen. The oxidizing operation may be carried on at substantially atmospheric pressure and at temperatures within the range of from about 300° F. to about 400° F., preferably in the presence of a catalyst such as the oxides of Mn, Cu, Fe, Cr and V, or the metals Cu, Fe, Cr and V, or the metal salts of organic acids such as copper or manganese oleates or naphthenates. While the oxidation may be carried on in the absence of a catalyst,

particularly at elevated pressures, it is desirable to employ a catalyst to increase the rate of the oxidation reaction. When the oxidizing operation is carried on at superatmospheric pressures, for example, pressures up to about 2000 lbs./sq. in., the temperatures required may be considerably lower than those employed at atmospheric pressure. Temperatures of the order of 200° F. to 300° F. are suitable when oxidation is effected at pressures of the order of 200 to 1000 lbs./sq. in., in the presence of one or more of the catalysts above mentioned. The choice of temperatures, pressures and time of contact to be employed in effecting oxidation is dependent upon the degree of oxidation and character of the products desired. The oxidizing operation may be carried on in a batch system, or a continuous system, wherein the oxidation products may be separated from the unconverted hydrocarbons and the latter recirculated for further treatment.

My invention may be further illustrated by the following example, but is in no wise limited thereto.

1 bbl. of tri-isobutylene (boiling range 340° F.—355° F.) together with 2.5% by weight of finely divided MnO<sub>2</sub> was charged to a suitable vessel provided with a vapor outlet and condenser. The mixture was continuously agitated and gradually heated, oxygen being bubbled through the liquid at a rate of about 4 cubic feet per minute. Oxidation reactions started at a temperature of about 260° F. with the formation of water, lower-boiling oily products and gas. These products were continuously distilled off as they were formed, separation from the reaction mixture being thus obtained. As the oxidation progressed, the temperature was increased to a maximum of 370° F., and the oxidation continued until no further oily distillate and water were obtained. The oily distillate was separated from the water, which latter was neutralized with sodium hydroxide and then treated with soda ash to effect a salting out of additional oily material. The initial oily distillate, after neutralization, was admixed with the oily material recovered from the aqueous distillate by the salting-out procedure, and the mixture was fractionally distilled to separate any unconverted tri-isobutylene. The oxidized, oily product thus obtained had a specific gravity of 0.82 at 60° F., a distillation range of from 144° F. to 327° F., an average molecular weight of 84, and contained 66.1% C, 13.1% H, and 20.8% O.

In order to determine the effectiveness of the tri-isobutylene oxidation product as an anti-

detonation agent for motor fuel, 25% by volume of the product as above described was blended with a straight-run gasoline and tested for anti-detonation value or octane number in accordance with the A. S. T. M.—C. F. R. Method D357-34T.

| Motor fuel                                                                | Octane number |
|---------------------------------------------------------------------------|---------------|
| Pennsylvania straight-run gasoline                                        | 41            |
| Pennsylvania straight-run gasoline+25% tri isobutylene oxidation products | 54            |

It will be seen from the above example that the oxidation products of tri-isobutylene, when blended with a hydrocarbon motor fuel, improves the anti-detonation value thereof to a marked degree. The oxidation products may be employed, per se, as motor fuel, or may be added to gasoline in any desired proportion, for example, 10%, 25%, 50% or more, depending upon the degree of improvement required. The blending of tri-isobutylene oxidation products is not necessarily confined to hydrocarbon motor fuels, since such oxidation products may be added to mixtures of gasoline and alcohol, gasoline and benzol, and the like. Other motor fuels, such as cracked gasoline and gasoline produced by the chemical or thermal polymerization of gaseous hydrocarbons, as well as straight run gasoline, may be improved by the addition of tri-isobutylene oxidation products.

What I claim is:

1. The method of increasing the anti-detonation characteristics of gasoline, which comprises adding to the gasoline an oxidation product of tri-isobutylene in an amount sufficient substan-

tially to increase its anti-detonation characteristics, said oxidation product boiling within the boiling range of gasoline and resulting from the oxidation of tri-isobutylene under conditions such that the ratio of oxygen to tri-isobutylene is at least mol for mol. 5

2. The method of increasing the anti-detonation characteristics of gasoline, which comprises adding to the gasoline an oxidation product of tri-isobutylene in an amount sufficient substantially to increase its anti-detonation characteristics, said oxidation product boiling within the boiling range of gasoline and resulting from the oxidation of tri-isobutylene at temperatures of from about 200° F. to about 400° F. and under 15 conditions such that the ratio of oxygen to tri-isobutylene is at least mol for mol.

3. A motor fuel of improved anti-detonation characteristics, comprising gasoline to which has been added an oily liquid oxidation product of tri-isobutylene boiling within the gasoline boiling range and resulting from the oxidation of tri-isobutylene under conditions in which the ratio of oxygen to tri-isobutylene is at least mol for mol. 20 25

4. A motor fuel of improved anti-detonation characteristics, comprising gasoline to which has been added an oily liquid oxidation product of tri-isobutylene boiling within the gasoline boiling range and resulting from the oxidation of tri-isobutylene at temperatures of from about 200° F. to about 400° F. and under conditions in which the ratio of oxygen to tri-isobutylene is at least mol for mol. 30

ERNEST M. MARKS. 35